

# UNITED STATES PATENT OFFICE.

FREDERICK M. BECKET, OF NIAGARA FALLS, NEW YORK, ASSIGNOR TO ELECTRO METALLURGICAL COMPANY, A CORPORATION OF WEST VIRGINIA.

## PROCESS OF PRODUCING LOW-CARBON, LOW-SILICON TITANIUM ALLOYS.

941,553.

Specification of Letters Patent. Patented Nov. 30, 1909.

No Drawing.

Application filed June 12, 1907. Serial No. 378,580.

To all whom it may concern:

Be it known that I, FREDERICK M. BECKET, a subject of the King of Great Britain, residing at Niagara Falls, in the county of 5 Niagara and State of New York, have invented certain new and useful Improvements in Processes of Producing Low-Carbon, Low-Silicon Titanium Alloys, of which the following is a specification.

10 When ores of titanium and an alloying metal are reduced by carbon in an electric furnace, the resulting titanium alloy contains a large proportion of carbon. Ferro-titanium high in carbon is not a desirable 15 alloy for use in the production of certain titanium steels. If, however, silica be added to the charge, the silicon reduced simultaneously with the titanium acts as a carbon-excluding agent and a low-carbon high-silicon 20 alloy may be produced.

According to the present process, a titanium alloy low in carbon and high in silicon is subjected to an oxidizing reagent for the 25 production of an alloy low in or substantially free from silicon. For example, the low-carbon high-silicon ferro-titanium produced by electrically smelting a charge containing oxids of titanium and silicon, carbon and a source of iron, is finely crushed and 30 mixed with iron oxid and the mixture is subjected to a temperature sufficient to effect the oxidation of silicon in the alloy with simultaneous reduction of the iron oxid, the reduced iron alloying with the ferro-titanium. 35 The iron oxid, for example hematite ore, may be added directly to the molten high-silicon alloy, either in the reduction furnace or in a separate vessel into which the alloy is tapped.

40 Iron oxid is a desirable reagent for removing the silicon from ferro-titanium; since it introduces no new constituent into the alloy. Oxids of other metals, reducible by silicon and alloyable with ferro-titanium, may obviously be employed.

The alloys produced by this process preferably contain titanium in excess of ten per cent., carbon not in excess of five per cent., and silicon not in excess of five per cent. A 50 product containing about 30% of titanium and 2% of carbon, substantially free from silicon, may be made by reacting with ferric-oxid on an initial alloy containing about 50% of titanium, 40% of silicon, 3% of car-

bon and 7% of iron. A product containing 55 30% of titanium and 5% of carbon, substantially free from silicon, may be similarly made from an alloy containing 41% of titanium, 22% of silicon, 7% of carbon and 30% of iron. For the production of forty per 60 cent. titanium, containing not more than 5% of carbon and substantially free from silicon, by the use of ferric-oxid as an oxidizer, an alloy is required containing 60% of titanium, 30% of silicon, 7% of carbon, and 3% 65 of iron.

I claim:

1. The process of producing low-silicon titanium alloys, which consists in producing a high-silicon titanium alloy and oxidizing 70 out the contained silicon.

2. The process of producing low-silicon titanium alloys, which consists in producing a high-silicon titanium alloy and oxidizing out the contained silicon by an oxid of the 75 alloyed metal.

3. The process of producing low-silicon ferro-titanium, which consists in producing high-silicon ferro-titanium and oxidizing out the contained silicon by means of iron 80 oxid.

4. The process of producing low-carbon, low-silicon, ferro-titanium, which consists in producing high-silicon ferro-titanium by 85 smelting a mixture of oxids of titanium and silicon, carbon and a source of iron, and oxidizing out the contained silicon.

5. The process of producing low-carbon, low-silicon, ferro-titanium, which consists in producing high-silicon ferro-titanium by 90 smelting a mixture of oxids of titanium and silicon, carbon and a source of iron, and oxidizing out the contained silicon by means of iron oxid.

6. The process of producing low-carbon, 95 low-silicon, ferro-titanium, which consists in electrically smelting a mixture of oxids of titanium and silicon, carbon and a source of iron, crushing the product and mixing it with iron oxid, and heating the mixture to a 100 temperature sufficient to effect the oxidation of silicon and reduction of iron.

In testimony whereof, I affix my signature in presence of two witnesses.

FREDERICK M. BECKET.

Witnesses:

CHAS. F. RANSOM,  
R. H. WARREN.